



quoise patinas may be provided by applying or brushing on dilute cupric nitrate, dilute ammonium acetate, dilute cupric carbonate, or dilute sodium thiosulphate and ferric nitrate. After burnishing, the metal coated clay object may be waxed and polished with a soft cloth.

When skillfully carried out, an oil based clay sculpture coated according to this invention will give the appearance of a bronze casting and will be a permanent art object.

The ingredients of the above coatings may be diluted in a suitable vehicle, e.g., water, and then cast in molds. After evaporation the hard formed articles can be shaped by machining and if not quite hard by pressure.

The end product from casting the above compositions into art objects for example, is lighter in weight than mere plaster of Paris with water. The product is tougher, harder, less brittle and less subject to chipping, breaking, crumbling, crazing or chalking than corresponding compositions of plaster of Paris with water.

The product cast from the present compositions can be coated easily by a mixture of polyvinyl acetate with powder, plaster of Paris and water. The powder in coating or casting may include metal particles to give a metallic character to the product. The particles are preferably about 40 to 350 mesh and may be bronze, copper, brass or a mixture of metals. Other metals of silver color such as aluminum may also be used.

Objects to be coated may be of wood, metal, concrete, plastic, clay, paper or ceramics. Structural elements such as blocks or the like may be coated for decorative effects. A metal plated appearance can thus be achieved. The coated product may be colored by inclusion or dyes, or colored powders such as metal oxides and may be antiqued. The object may be polished, smoothed or burnished after coating.

Further examples of the invention are as follows:

#### CASTING MATERIALS AND PLATING MATERIALS

The products used for this new, novel casting (molding) material are:

40 to 60% by volume of fine mesh plaster of Paris mixed with 40 to 60% by volume of wood flour (microporous cellulose) 150 mesh or finer. Mix these two powders dry.

Add polyvinyl acetate emulsion, dilute with water (by volume from 25 to 60%).

I have found that a polyvinyl acetate emulsion diluted with water in the ratio of 60% PVA and 40% water or 50% each by volume added to above mixed powders makes a most satisfactory casting material as to setting time, amount of hardness, toughness, and other qualities expressed above in my description of castings.

Water is cheaper than the polyvinyl acetate emulsion, but this emulsion is the binder, additive or catalytic agent that creates a new material.

There is a chemical reaction between the polyvinyl acetate diluted with water and the plaster of Paris, and a reaction of the wood flour and the adhesive qualities of the polyvinyl acetate solution.

The powders and the diluted PVA emulsion are mixed in a container.

The liquid mixture is either

(1) Cast in a mold.  
(2) Applied to any hard surface or object by brush or air spray.

(3) When casting, the mixture of the powders and the polyvinyl acetate emulsion should be prepared in sufficient quantity for the size or volume needed for the job.

(4) Allow the casting to dry and cure before removing from the mold.

(5) Any imperfections in the surface of the casting, can be easily remedied or repaired with the application of a small amount of newly made batch of casting material.

(6) Before casting is completely hard or cured, any irregularities or imperfections may be easily trimmed with a knife.

(7) Hardened castings can be sandpapered. It is advisable to do this before complete curing.

Process of plating or coating ceramic objects, clay, wood, plastic, metal, plaster of Paris, or any other object where electroplating is not practical or feasible

10 Objects can be plated or coated with powdered metals such as bronze, brass, copper, aluminum, etc. and/or for direct color effects dry color powders may be added, also silic acid and metal oxides.

#### (I) BRONZE (NON-FERROUS) PLATING OF OBJECT

A bronze metallic electrolytic powder is used for plating. The mesh of the metal powder can be from about 40 mesh to 325 mesh.

The finish desired will determine the number mesh needed. For a most practical smooth bronze plating finish, I have used 150 mesh. For rough texture I have mixed or added heavier mesh bronze powders, and brass key filings may be added. Copper or brass can be added or substituted. These mixtures or combinations of metals and meshes will depend on the desired "End Resultant Finish."

#### (II) PREPARATION AND APPLICATION OF PLATING MIXTURE

(A) Dry mix 1 part of plaster of Paris (fine) with 1 part of wood flour (described above).

(B) Add this dry mixed powder to the bronze metal powder in this proportion: 1 part volume mixed powder 35 4 parts volume bronze metal powder.

(C) Dry mix thoroughly.

(D) Add P.V.A. emulsion previously diluted with water 50/50 so resultant mixture has the consistency of heavy cream.

40 (E) Mix thoroughly and apply to object with brush. Apply with steady stroke. This plating material hardens rapidly. The container and brush must be washed in water after each use.

(F) Several coats of this metal powder, gypsum, wood flour and polyvinyl acetate emulsion will provide a very hard, durable and dense metallic coating.

#### (III) FINISHING AND PATINA OF PLATED OBJECT

(A) When object has hardened, dried and is completely cured, object may be sanded with fine sandpaper wherever high lights are desired, or where the sheen of cast polished bronze is wanted.

55 (B) Patina or antiquing bronze plated object.—The non-ferrous metal plated object can now be antiqued or colored, in part or whole, depending on the finish desired.

(1) To turn the non-ferrous plating to black or deep brown finish quickly, apply a small amount of ammonium sulphide by hair brush or Q tip. Dilute with water for lighter color effects. I have found that vapors of concentrated solution of ammonium sulphide, which are heavy will color copper a beautiful burnt orange or red, as you pass over object and touch lightly in spots.

(2) For green antiqued patina, mix acetic acid, or citric acid, or ammonium acetate with malachite (copper carbonate), add a small amount of polyvinyl acetate emulsion. Apply with brush and allow to dry. The chemical reaction for a real antique finish takes a few days. Repeat if darker effects are necessary.

(3) To antique brass, simply cover with a solution of antimony chloride and allow to dry.

(4) For blue green bronze apply a solution of sodium thiosulfate and ferric nitrate.

- (5) For intense green, mix acetic acid and copper nitrate 50/50. Apply and allow to dry. Chemical reaction will be complete in a few days. I have used different amounts of acetic acid and ammonium acetate, copper nitrate and malachite mixed together and applied to object. Unusual antique effects.
- (6) When the desired colors or combination of colors have dried and are set, the object should be sanded lightly to bring out the metallic bronze sheen.
- (7) Object can be burnished, waxed or polished with soft cloth.

(C) Finish.—When skillfully carried out, the plating and the application of the chemicals for a patina, the object has a realistic appearance, weight, feel of an expensive casting at a fraction of the cost.

The casting has now become a durable, permanent art object.

What is claimed is:

1. The process of coating a shaped object comprising the steps of:
- (a) preparing a dry powder mixture comprising wood flour and plaster of Paris;
  - (b) dusting the object with the dry powder mixture;
  - (c) rubbing the dry powder mixture dusted onto the object into its surface;
  - (d) removing excess powder from the surface of the object;
  - (e) preparing a liquid mixture of wood flour and plaster of Paris in water with polyvinyl acetate;
  - (f) painting the surface of the powder coated object with the liquid mixture; and
  - (g) allowing the painted surface to cure to provide a hardened coating and permanence for the coated object.

2. The process according to claim 1 wherein in steps (a) and (e) wood flour and plaster of Paris are mixed in substantially equal parts by volume.
3. The process according to claim 2 wherein successive coats of the liquid mixture are painted on the surface of the object and allowed to cure between coats.
4. The process according to claim 2 with the additional step of further finishing the coated object by painting it with a conventional hard drying covering.
5. The process according to claim 2 with the additional steps of:
- (h) preparing a second liquid mixture of a fine metal, wood and gypsum powder in water with polyvinyl acetate;
  - (i) painting the object with the second liquid mixture; and
  - (j) allowing the painted surface to cure.
6. The process according to claim 5 wherein the fine metal powder is bronze and with the additional steps of:
- (k) chemically forming a patina on the metal covered surface of the object; and
  - (l) burnishing the patina revealing the metal surface therebelow where desired.
7. An object coated by the method of claim 1.

#### References Cited

##### UNITED STATES PATENTS

3,558,340 1/1971 Spector ----- 117—26

30 WILLIAM D. MARTIN, Primary Examiner  
R. M. SPEER, Assistant Examiner

U.S. Cl. X.R.

35 35—26; 117—16, 29; 264—131